

Jan. 10, 1939.

G. F. NADEAU

2,143,791

PHOTOGRAPHIC STRIPPING FILM

Filed May 16, 1936

FIG. 1.



FIG. 2.



FIG. 5.



FIG. 3.



FIG. 4.



FIG. 6.



INVENTOR.

Gale F. Nadeau

By  
Newton M. Perrins  
R. Frank Smith  
ATTORNEYS

## UNITED STATES PATENT OFFICE

2,143,791

## PHOTOGRAPHIC STRIPPING FILM

Gale F. Nadeau, Rochester, N. Y., assignor, by  
mesne assignments, to Eastman Kodak Com-  
pany, Jersey City, N. J., a corporation of New  
Jersey

Application May 16, 1936, Serial No. 80,127

9 Claims. (Cl. 95—9)

This invention relates to photographic strip-  
ping film, that is, film in which the sensitive layer  
is carried on a temporary support from which it  
may be removed, together with a permanent sup-  
port layer, after exposure.

A photographic stripping film of this type is  
described, for example, in U. S. Patent No. 1,973,-  
476 of Fordyce et al. These films are used in the  
photo-engraving and related arts where an image  
is to be recorded and after development and fix-  
ing, removed from the temporary support and  
affixed to a transparent plate for the purpose of  
making photo-engraving plates. The emulsions  
used are usually a type which give an image hav-  
ing a high degree of contrast. A frequent diffi-  
culty encountered in this type of film is the pres-  
ence of areas of varying sensitivity, produced by  
the lack of uniformity of overlying layers or by  
other factors, not fully understood. This results  
in the formation of undesirable lines and mottle  
on the negative. A method of overcoming these  
undesirable factors was described in my prior ap-  
plication, Serial No. 64,103, filed February 15,  
1936, in which I described an adhesive layer hav-  
ing a controlled hydrogen ion concentration so  
that the emulsion layer would not be adversely  
affected.

The principal object of the present invention is  
to provide an improved method for overcoming  
these difficulties and for producing a stripping  
film in which the sensitive emulsion does not show  
areas of varying sensitivity.

This object is accomplished by applying a layer  
of cellulose ester or synthetic resin to the tem-  
porary support and coating the adhesive over  
this cellulose ester or synthetic resin layer. Ex-  
perimentation has established the fact that much  
of the above-mentioned difficulty may be attrib-  
uted to the unevenness and lack of uniformity of  
the adhesive layer. When the adhesive is ap-  
plied directly to the paper temporary support it  
is differentially imbibed by the paper stock. By  
applying a layer of cellulose ester or synthetic  
resin over the paper stock between the paper and  
the adhesive layer, this absorption of the adhe-  
sive by the paper is prevented, with the result  
that very much less adhesive need be used and a  
uniform coating is obtained.

In the accompanying drawing which forms a  
part of the present invention I have shown a num-  
ber of enlarged sectional views of stripping film  
made according to my invention.

Fig. 1 is a sectional view of a stripping film  
having a layer of cellulose ester between the paper  
support and the adhesive layer.

Fig. 2 is a sectional view of a similar type of  
film having cellulose ester and gelatin layers ap-  
plied to the reverse side of the paper support.

Fig. 3 is a sectional view of a stripping film in  
which a layer of synthetic resin is applied be-  
tween the paper support and the adhesive layer.

Fig. 4 is a sectional view of a stripping film in  
which a layer of a water-soluble synthetic resin  
is applied between the paper support and the per-  
manent emulsion support.

Fig. 5 is a sectional view of a film similar to  
that shown in Fig. 1, but having an anti-halation  
dye in the baryta coating of the paper temporary  
support.

Fig. 6 is a sectional view of a film similar to  
that shown in Fig. 1 but having a transparent  
cellulose ester temporary support and an anti-  
halation backing layer.

The construction of the stripping film accord-  
ing to my invention will now be described by par-  
ticular reference to the accompanying drawing.  
As shown in Fig. 1, the support 10, which is a  
temporary support of paper or other suitable ma-  
terial, is coated with a layer 11 of a cellulose  
ester, such as cellulose nitrate or cellulose ace-  
tate, or a mixed ester, such as cellulose acetate  
propionate. The composition of this ester is not  
critical. The cellulose ester is applied from a 5  
to 10% of the ester in solution in a suitable sol-  
vent. This solvent may be a mixture of 85% 30  
methyl alcohol and 15% acetone, or pure acetone,  
methyl Cellosolve or other solvent. Over this  
ester layer 11 there is applied a thin gelatin sub-  
layer 12. The composition of the gelatin solution  
from which this layer is applied may be as fol-  
lows:

|               | Grams |
|---------------|-------|
| Gelatin       | 1.2   |
| Acetic acid   | 1.2   |
| Acetone       | 70 40 |
| Water         | 5     |
| Ethyl alcohol | 22.6  |

The adhesive layer 13 is applied next. This  
layer may consist of a 10 to 15% aqueous solution  
of water-soluble glue or a mixture of 8% liquid  
glue and 8% glycerine in 84% of water. The per-  
manent support layer 14 is then applied over the  
adhesive layer. This permanent support layer  
may consist of cellulose nitrate or acetate or other  
cellulose ester. I prefer to use, however, a cellulose  
nitrate of low nitrogen content and high al-  
cohol solubility. A cellulose nitrate of this com-  
position should contain approximately 9 to 12%  
of nitrogen and have a solubility in methyl alco- 55

hol of 30% to 100% and a viscosity of 2 to 5 seconds by the dropping ball method. This cellulose nitrate should be water permeable in order to permit the water of the developing bath or other treatment baths to reach and penetrate the adhesive layer. In order to increase this water permeability, it is desirable to add certain materials, such as glyceryl Boric-borate (sold by Glyco Products Company, New York, N. Y.), mono-, di- and tri-acetin, lactic acid, glycerine, various triethanolamine derivatives, lithium chloride, cadmium bromide or other materials. The nitrate may be applied in a solution of 7½% nitrate in methyl alcohol, acetone and butyl alcohol or similar solvents. The gelatin sub-layer 15 is applied next and is followed by the emulsion layer 16. The gelatin layer 15 may be applied from a solution having the same composition as the gelatin layer 12.

20 Viscosity by the dropping ball method referred to above is determined as follows:

10 grams of dry nitrocellulose are dissolved in 100 cc. of a mixture comprising 50% by volume of methyl alcohol and 50% by volume of acetone at 25° C. Viscosity is measured by the time in seconds it takes for a steel ball having a diameter of  $\frac{1}{8}$ th of an inch and weighing .1320 to .1340 grams to fall 15 centimeters through the nitrocellulose solution at 25° C. in a tube having a diameter of  $1.7 \pm .05$  centimeters.

As shown in Fig. 2 the paper support 10 is coated on one side with the layers 11, 12, 13, 14, 15 and 16 as described above. On the opposite side of the paper support 10 there is coated a layer 17 of a cellulose ester, such as nitrate or acetate which may have the same composition as the layer 11. Over this layer 17 there is coated a gelatin layer 18. The purpose of these layers is to prevent curling of the element prior to or during exposure and to prevent water absorption by the paper support during processing. The cellulose ester layer 17 prevents penetration of water to the paper support 10 and the layer 18 aids in counteracting the curling tendency of the film and causes it to lie flat.

45 In the modification of my invention shown in Fig. 3 a layer of a synthetic resin which is not easily attacked by water is substituted for the cellulose ester layer applied to the paper support. 50 As shown in this figure the paper support 10 is coated with a layer of a synthetic resin 19. This is applied from a 3 to 10% solution of the resin in an appropriate solvent, such as ethylene chloride, acetone, or a mixture of ethylene chloride and methyl alcohol or acetone and methyl alcohol. Over the resin layer 19 there is applied a thin protective layer 20 of a cellulose ester, such as cellulose nitrate. This layer is applied merely to prevent the resin layer 19 from sticking in the 55 parts of the coating machine through which it passes. The cellulose ester layer 20 is followed by the gelatin sub-layer 12 as described above and over this is coated the layers 13, 14, 15 and 16, as previously described.

60 Among the synthetic resins which may be used in stripping film according to my invention, a great many materials are available. These include the polyvinyl esters, such as polymerized vinyl acetate which is shown, for example, under 65 the tradename "Gelva", the preparation of which is described in the U. S. Patent Nos. 1,241,738; 1,586,803 and 1,710,825. A further type of resin which may be used is the polyvinyl acetal type. These resins are condensation products of partially or completely hydrolyzed polyvinyl acetate

and an aldehyde, such as formaldehyde, acetaldehyde, or butyraldehyde and are known as polyvinyl acetals. They are sold under various trade-names such as "Formvar" and "Alvar", the preparation of which is described in British Patent No. 351,082 and in U. S. Patent Nos. 1,955,068 and 1,990,399. A still further type of resin which I may use are the alkyd resins, which are condensation products of a polybasic acid and a polyhydroxy alcohol. An example of this type of resin is "Glypta", which is a condensation product of glycerine and phthalic acid or phthalic anhydride. A still further type of resin is the group known as the "Santolites" which are condensation products of formaldehyde with aromatic sulfonamides.

I have also discovered that the adhesive layer may be partially or completely eliminated and in its place a water-soluble resin, such as polyvinyl alcohol applied to the paper support. A film of this type is shown in Fig. 4. As shown in this figure the paper support 10 is coated with a layer 21 of polyvinyl alcohol in a 3 to 10% solution in water. The concentration of this solution will be determined by the method of application and by the speed of the coating operation. A thin layer 22 of cellulose nitrate is applied over the polyvinyl alcohol layer and is followed by a heavier layer 23 of cellulose nitrate or of cellulose acetate or other cellulose ester which constitutes the permanent support. This is followed by the sublayer 15 and emulsion layer 16.

In the modification of my invention in which a water-soluble synthetic resin is used as the adhesive layer, it is sometimes desirable to coat a thin layer of a water-soluble glue directly over the resin layer. This is coated as a very thin layer, much thinner than where the glue is used as the only adhesive, and may be, for example, a 2% solution of glue containing 1% of glycerine in water. The advantage of a stripping film in which the glue layer is partially or completely eliminated is that the stripping time is considerably reduced since the water of the processing bath does not need to penetrate a heavy glue layer.

As shown in Fig. 5 the film may contain an anti-halation dye to prevent reflection of light from the paper support. As shown in this figure the paper support 10 has a baryta coating 24 containing the anti-halation dye. This anti-halation layer is coated with the cellulose ester layer 11 followed by the gelatin sub-layer 12, the adhesive layer 13, the permanent support layer 14, the gelatin sub-layer 15 and the emulsion layer 16.

It is also possible to apply the cellulose ester intermediate layer used according to my invention to a support layer of transparent material, such as a cellulose ester, instead of to the paper support. As shown in Fig. 6 the cellulose acetate temporary support layer 25 is coated with a cellulose nitrate or acetate layer 11 and this is followed by the gelatin sub-layer 12, the adhesive layer 13, the permanent support layer 14, the gelatin sub-layer 15 and the emulsion layer 16. On the opposite side of the transparent temporary support 25 there may be coated an anti-halation layer 27 of gelatin containing manganese dioxide or other suitable anti-halation material, coated over a subbing layer 26 of cellulose nitrate or other cellulose ester. This anti-halation backing may, of course, be omitted. The advantages of a transparent temporary support layer are that the operator may view the negative during processing and determine the extent of the develop-

ment. A film having a temporary support layer of a cellulose ester is light in weight and not liable to breakage prior to use.

A photographic stripping film having a cellulose layer between the temporary support and the adhesive layer has a number of important advantages. Such a film is free from emulsion difficulties, such as lines and mottle and also may be stripped from the temporary support more easily and quickly than with films used hitherto. Less adhesive may be used and there is a consequent decrease in the stripping time since less water must diffuse through the layers to dissolve the reduced quantity of adhesive.

15 Although I have described a certain sequence of layers in the stripping film according to my invention, it is to be understood that not all of these layers are absolutely essential and that other layers may be added if desired. The essential feature of my invention is the use of a cellulose ester or synthetic resin layer between the temporary support and the adhesive layer, or the substitution of a water-soluble resin layer for the adhesive layer. The remaining layers are added 20 in a manner well known to those in the photographic film-making art. It is known, for example, that a gelatin layer does not readily adhere to a cellulose acetate layer of every composition, although the gelatin layer will adhere to a cellulose nitrate layer. In some cases it is necessary to use an additional layer between the cellulose acetate and the gelatin layer in order to 25 secure satisfactory adherence. The paper support may also carry other layers, such as a baryta or dextrin coating or both. My invention is to 30 be taken as limited only by the scope of the appended claims.

What I claim is:

1. A photographic stripping film comprising a 40 temporary support, a water-permeable cellulose ester permanent support having a sensitive emulsion layer thereon, and between said temporary support and said cellulose ester permanent support, separate layers of a water-insoluble synthetic organic colloidal material and a water-soluble adhesive, the former layer being adjacent 45 the temporary support, and said layers adhering firmly in the dry state.

2. A photographic stripping film comprising a 50 temporary support, a water-permeable cellulose ester permanent support having a sensitive emulsion layer thereon, and between said temporary support and said cellulose ester permanent support, separate layers of a water-insoluble cellulose ester and a water-soluble adhesive, the former 55 layer being adjacent the temporary support, and said layers adhering firmly in the dry state.

3. A photographic stripping film comprising a

temporary support, a water-permeable cellulose ester permanent support having a sensitive emulsion layer thereon, and between said temporary support and said cellulose ester permanent support, separate layers of synthetic resin and a water-soluble adhesive, the former layer being adjacent 5 the temporary support, and said layers adhering firmly in the dry state.

4. A photographic stripping film comprising a temporary support, a water-permeable cellulose 10 ester permanent support having a sensitive emulsion layer thereon, and between said temporary support and said cellulose ester permanent support, separate layers of cellulose nitrate and a water-soluble adhesive, the former layer being 15 adjacent the temporary support, and said layers adhering firmly in the dry state.

5. A photographic stripping film comprising a paper support, a cellulose ester layer on each side of said paper support, and in order on one of said cellulose ester layers, a water-soluble adhesive 20 layer, a transparent water-permeable permanent support layer, and a photographic emulsion layer, all of said layers adhering firmly in the dry state.

6. A photographic stripping film comprising a paper support, a cellulose nitrate layer on each side of said paper support, and in order on one of said cellulose nitrate layers, a water-soluble adhesive layer, a transparent water-permeable permanent support layer, and a photographic emulsion 25 layer, all of said layers adhering firmly in the dry state.

7. A photographic stripping film comprising a paper support, a cellulose ester and gelatin layer 30 in order on each side of said paper support, and in order on one of said gelatin layers, a water-soluble adhesive layer, a transparent water-permeable permanent support layer, and a photographic emulsion layer, all of said layers adhering firmly in the dry state.

8. A photographic stripping film comprising a temporary support, a water permeable cellulose ester permanent support having a sensitive emulsion layer thereon, and between said temporary support and said cellulose ester permanent support, separate layers of a water-insoluble cellulose ester and a water-soluble adhesive, the former 45 layer being adjacent the temporary support, and said layers adhering firmly in the dry state.

9. A photographic stripping film comprising a 50 paper support, on one side of said paper support successive layers of cellulose ester, water-soluble adhesive, transparent water-permeable cellulose ester permanent support, and sensitive emulsion, and on the opposite side of said paper support, a 55 layer of an organic acid ester of cellulose.

GALE F. NADEAU.